# EUROPEAN PATENT SPECIFICATION

(11) **EP 0 073 125 B1**
(45) Date of publication and mention of the grant of the patent: **05.03.1986**
(21) Application number: 82304282.5
(22) Date of filing: 13.08.1982
(51) Int. Cl.: G21F 9/34

(54) **Method of encapsulating spheroids containing nuclear waste**
Verfahren zum Überziehen von Spheroiden die nukleare Abfälle enthalten
Méthode pour enrober des sphéroides, contenant des déchets nucléaires

(30) Priority: 14.08.1981 US 293047
(43) Date of publication of application: 02.03.1983
(73) Proprietor: WESTINGHOUSE ELECTRIC CORPORATION, Pittsburgh Pennsylvania 15222 (US)
(72) Inventor: Pope, James Michael, Monroeville Pennsylvania (US); Harrison, Don Edward, Murrysville Pennsylvania (US)
(74) Representative: Marchant, James Ian

## Description

This invention relates to a method of encapsulating spheroids containing nuclear waste.

Approximately 25 million gallons of high-level nuclear waste has accumulated at the Savannah River Laboratory (SRL) of the Department of Energy (DOE) from the production of defense materials during the past 25 years. One procedure under consideration for disposing of this nuclear waste is to encapsulate it in glass or ceramic spheroids. The spheroids are then coated to reduce the leachability of the nuclear waste from the glass material. The coated glass or ceramic spheroid waste form concept is one having particular appeal because the spherical waste form is produced directly from a liquid in a dustless process that is especially amenable to remote operation. However, the procedures planned for coating the spheroids pose some serious difficulties because three separate coatings are to be applied by chemical vapor deposition at temperatures greater than 1100°C. First, pyrolytic carbon will be deposited by thermal decomposition of acetylene in a fluidized bed reactor. Then, two alumina layers will be applied by using gaseous aluminum tetrachloride and hydrogen in a rotating drum furnace. The use of highly combustible gases and high temperatures in combination with nuclear waste creates a danger of an explosion or fire with the -potential release of radionuclides. Also, complex manipulations must be performed by remote operations, and hydrochloric acid by-product solutions are produced which are difficult to treat.

We have discovered a method of applying an amorphous coating to glass or ceramic spheroids containing nuclear waste. The coating is of very low leachability and can be made to have about the same thermal expansion as the spheroids do, so that cracking does not occur with changes in temperature. The coating can be applied and cured at temperatures of from 400 to 500°C, but if desired, it can be heated at about 850°C to give a dense amorphous coating of the same quality as coatings produced conventionally at much higher temperatures.

Our prior European Patent Application Publication No. 0042770 A2 relates to a method of immobilizing nuclear waste characterized by (A) preparing a composition which comprises (1) from 60% to about 100% by weight, calculated as Si0₂, of a hydrolyzed silicon compound having the general formula or where each R is independently selected from alkyl to C₁₀ and alkenyl to C₁₀, each R' is independently selected from R and aryl, each X is independently selected from chlorine and bromine, m is 0 to 3, n is 0 to 4, p is 0 to 1, and m+n+p equals 4; (2) up to about 40% by weight, calculated as AI₂0₃, of an aluminium compound having the general formula or where each R is independently selected from alkyl to C₁₀ and alkenyl to C₁₀, each R' is independently selected from R or aryl, q is 0 to 3, r is 0 to 3, s is 0 to 1, and q+r+s equals 3; (B) mixing from 1 to 50% based on total weight, of said nuclear waste in liquid form into said composition; (C) mixing up to about 10%, based on total weight, of said nuclearwaste in solid form into said composition; and (D) heating said composition containing said nuclear waste at from 200 to 500°C to drive off water and organics.

This method is for immobilizing liquid and solid nuclear wastes by mixing them with a composition which is somewhat similar to that used as the coating composition according to the present invention, although there are differences in the percentages ranges of the silicon and aluminium compounds. The present invention is confined to the treatment of nuclear waste already contained in glass or ceramic spheroids.

The present invention provides a method of encapsulating glass or ceramic spheroids containing nuclear waste characterized by (A) dropping the spheroids individually into a coating apparatus; (B) coating the spheroids in the coating apparatus with a composition which comprises (1) from 30% to 85% by weight, calculated as Si0₂, of a partially hydrolyzed silicon compound having the general formula or where each R is independently selected from alkyl to e₁₀ and alkenyl to Cᵢₒ, each R' is independently selected from R and aryl, each X is independently selected from chlorine and bromine, m is 0 to 3, n is 0 to 4, p is 0 to 1, and m+n+p equals 4; (2) up to about 30% by weight, calculated as AI₂0₃, of a partially hydrolyzed aluminium compound having the general formula or where each R is independently selected from alkyl to C₁₀ and alkenyl to C₁₀, each R' is independently selected from R and aryl, each X is independently selected from chlorine and bromine, q is 0 to 3, r is 0 to 3, s is 0 to 1, and q+r+s equals 3, and (3) from 30 to 50 percent by weight of an alcohol; (C) hardening the coatings on the spheroids whilst preventing the coated spheroids from one another; and touching the coatings by heating the coated spheroids in air to a temperature of up to 850°C.

In order that the invention can be more clearly understood, convenient embodiments thereof will now be described, by way of example, with reference to the accompanying drawings in which:
Figure 1 is a diagrammatic side view, in section, illustrating a spraying process for coating spheroids, and Figure 2 is a diagrammatic side view, in section, showing a two-liquid immersion process for coating spheroids. Alternatively, this two-liquid immersion process could alo be utilized in reverse provided the specific gravities of the constituent fluids were properly matched.

Referring to Figure 1, a sphere dispenser 1 drops spheroids 2 one at a time into chamber 3. At the top portion of the chamber, spray nozzles 4 spray a coating composition according to this invention onto spheroids 2. In the lower portion of chamber 3 a heating coil 5 heats the coatings 6 on the spheroids and hardens them.

In Figure 2, a sphere dispenser 7 drops spheroids 8 one at a time into trough 9. The trough 9 contains a hydrolyzed alkoxide coating composition 10 in its upper portion, an immiscible liquid layer 11 in its middle portion, and a hardening agent 12 in its lower portion.

The immiscible liquid layer, which separates the coating composition from the hardening agent, is necessary because otherwise the two fluids will mix and the entire coating composition will become hard. A silicone oil layer 3,17 to 6,35 mm (1/8 to 1/4 inch) thick has been found suitable for this purpose. It is preferable to heat the hardening fluid up to about 75°C to accelerate the hardening process. Higher temperatures, however, should be avoided as they may result in bubbles in the coating. A pump 13 circulates the hardening fluid through line 14 which forces the coated spheroids up tube 15 onto moving belt 16 into heated chamber 17. Excess hardening fluid is collected in vessel 18 where it passes through line 19 to the pump for recirculation. In heated chamber 17 the coated spheroids are calcined to glassify the coating. The spheroids then pass through opening 20 where they are collected for disposal.

In the two liquid-immersion process the hardening fluid may be either a setting ("electrolytic") agent or a dehydrating agent. Sodium hydroxide, ammonium hydroxide, hydrochloride acid, acetic acid, and hot water, are suitable setting agents. Sodium hydroxide is preferred because it promotes the most rapid hardening, although it does contaminate the coating somewhat with sodium ions. The purpose of the hardening agent is to make the coating sufficiently hard and non-tacky so that the spheroids will not stick together and the coating will not be damaged in handling. The amount of setting agent required to produce hardening of the coating may vary from 0.03 to 0.1 moles per mole of alkoxide glass forming constituent. Generally, equal volumes of alkoxide coating solution and setting agent are present in the system when sodium hydroxide is used as the setting agent. With the other setting agents which take a longer time for hardening, about 3 to 4 times as much as the coating solution is used to give an increased travel time.

The dehydrating agent works by removing water from the alkoxide composition, thus further cross-linking the silicon and aluminum oxides. The preferred dehydrating agent is trichloroethylene as it has been found to work well, although 2-ethyl-1-hexanol or octanol may also be used. When a dehydrating agent is used, a molecular sieve should be inserted into the recirculating line leading from the pump to remove the water captured by the dehydrating agent. It is preferable to use a dehydrating agent instead of a setting agent as dehydrating agents do not introduce contaminant species such as sodium into the coating, even though they promote less rapid hardening of the coating.

The final step in the process of this invention is to cure the coating which can be accomplished by heating the coated spheroids to 400 to 500°C in air for about one hour. At this temperature the cured coating contains closed porosity. Heating to about 800°C will completely densify the coating. To avoid thermal shock it is desirable to expose the coated spheroids to a temperature of about 100°C before exposing them to the higher temperature.

The process of this invention may be repeated using the same spheroids in order to enhance the thickness of the coating to the desired level. Generally, a coating of about 0.5 mm thick is considered desirable for the disposal of nuclear waste. Each coating cycle, however, should not add more than about 0.1 mm to the thickness of the coating in order to avoid cracks in the coating. Preferably, each cycle should add about 0.05 mm to the coating thickness. This normally means from 5 to 10 passes are required to produce a coating of a desired thickness.

The nuclear waste contained in the spheroids may take a variety of forms such as a sludge consisting of a mixture of complex hydroxides or hydrolyzed oxides of aluminum, iron, magnesium, manganese, silicon, calcium, sodium, potassium, ruthenium, mercury, nickel, cesium, strontium, uranium, molybdenum, the transuranics, and other elements. Defense nuclear waste can also include up to about 10 percent by weight sulfate, phosphate, nitrate, or mixtures thereof, and up to about 95 percent by weight water. The radioactive elements in nuclear waste may include uranium, thorium, cesium, ruthenium, iodine, and strontium. The nuclear waste in the spheroids may also be the result of fuel reprocessing which produces an aqueous nitrate solution of many of these elements.

The nuclear waste is contained in various types of glass or ceramic, usually of a borosilicate type by processes well known in the art. See, for example, the reference "Ceramics in Nuclear Waste Management", Proceedings of an International Symposium held in Cincinatti, Ohio, April 30-May 2, 1979, sponsored by the American Ceramic Society and the U.S. Dept. of Energy, pp. 73-122. There are several basic processes for containing the nuclear waste in spheroids. One process is a gel precipitation process. In this process the nuclear waste is mixed with a gel-support additive such as polyvinyl chloride, methyl cellulose, and/or formamide. Drops of the mixture are then permitted to fall into a gelation agent, such as ammonium hydroxide, which hardens the drops into small spheroids. The spheroids are then collected and are heated to remove the organics and to densify them, resulting in ceramic spheroids about 0.5 to about 3 mm diameter.

Another process for containing the nuclear waste in spheroids is a marble process. In this process nuclear wastes are mixed with glass frit containing such constituents as sodium oxide, silicon dioxide, and boron oxide. The mixture is then melted and cast into molds. This process produces glass spheroids from 10 to 25 mm in diameter.

The spheroids should be cleaned before they are used in the process of this invention. Cleaning may be accomplished by immersion in trichloroethylene, ethyl alcohol, one molar (1 M) nitric acid, or other cleaning fluids.

The composition used to coat the glasses is a mixture of alcohol and partially hydrolyzed alkoxides. The first glass-forming component of the composition is prepared from a silicon compound having the general formula or where each R is independently selected from alkyl to e₁₀ and alkenyl to Cᵢₒ, each r' is independently selected from R and aryl, each X is independently selected from chlorine and bromine, m is 0 to 3, n is 0 to 4, p is 0 to 1, and m+n+p equals 4. The compounds are preferred due to their availability, stability and compatibility with the other glass-forming constituents. The R' group is preferably alkyl to C₄ with n=4 because these alkoxides are the most suitable starting compounds.

Examples of appropriate compounds which fall within the scope of the general formula include:

The preferred silicon compound is tetraethylorthosilicate because it is relatively inexpensive, readily available, stable, and easy to handle. Before the silicon compound is added to the composition, it is partially hydrolyzed because its rate of hydrolysis is slower than the other compounds, and preferential precipitation may result if the components are hydrolyzed after they have been combined. Partial hydrolyzation may be accomplished by the addition of water to the silicon compound, where either the water, the silicon compound, or both, have been diluted with alcohol. The molar ratio of a silicon compound to the alcohol can range from 0.2 to 2. The alcohol is preferably the same alcohol that is produced during hydrolyzation so that it is not necessary to separate two different alcohols. The mole ratio of the silicon compound to the water can range from 0.1 to 5. It is occasionally necessary to use up to about six drops of concentrated nitric acid per mole of water to aid in the hydrolyzation reaction.

The second component of the composition is an aluminum compound which has a general formula or where each R is independently selected from alkyl to e₁₀ and alkenyl to Cₗₒ, each R' is independently selected from R and aryl, q is 0 to 3, r is 0 to 3, s is 0 to 1, and q+r+s is 3. The compounds, where r is 3 and R is alkyl to e₄ are preferred as they are the most stable and available and are easiest to handle. Examples of suitable aluminum compounds include:

The preferred aluminum compound is aluminum secondary butoxide because it is stable, available, and does not require special handling. These compounds are hydrolyzed prior to addition to the composition to avoid inhomogeneities. Hydrolysis can be accomplished using a molar ratio of aluminum compound to water of from 0.0007 to 0.03 and using from 0.03 to 0.1 mole of 1M HN0₃ per mole of AIO(OH) produced. The water is preferably heated to from 70 to 100°C.

In addition, the composition may contain alkoxides of boron or sodium which may be needed to match the thermal expansion of the coating with the thermal expansion of the spheroids. However, preferably no boron or sodium compounds are present as they increase the leachability of the coating. Sodium compounds which could be used have a general formula NaOR or NaZR'₃ where each R is indepenently selected from alkyl to C₁₀ and alkenyl to Cᵢₒ, each R' is independently selected from R and aryl, and Z is carbon or boron. The NaOR compounds where R is alkyl to C₄ are preferred as they are more stable and compatible. The sodium compounds should be hydrolyzed prior to being mixed into the composition to avoid differential hydrolyzation. A molar ratio of a sodium compound to water of from 0.003 to 0.1 may be used for hydrolyzation. Suitable sodium compounds which fall within the scope of the general formula include:

Sodium methylate is preferred as it is easier to handle and is readily available.

Boron compounds which can be used have a general formula where each R is independently selected from alkyl to e₁₀ and alkenyl to C₁₀, each R' is independently selected from R and aryl, q is 0 to 3, r is 0 to 3, s is 0 to 1, and q+r+s is 3. The compounds where R is alkyl C₄ and r is 3 are preferred as they are relatively available and well-matched with the other constituents. A molar ratio of a boron compound to water of from 0.1 to 1.0 may be used. Dilution in the same alcohol as that of the boron compound at a level of from 15 to 25 moles alcohol to boron compound is preferred for a more homogeneous hydrolyzation. Suitable boron compounds which fall within the scope of the general formula include:

Trimethylborate and triethylborate are preferred as they are relatively available and are compatible and require very little special handling.

Finally, the composition preferably includes up to about 2 percent of a surfactant to increase the adhesion of the coating to the spheroid. A suitable surfactant is octylphenoxypolyethoxy- ethanol sold under the trade designation Triton X-102 by Rohm and Haas of Philadelphia, Pennsylvania.

The invention will now be illustrated with reference to the following Examples:

### Example 1

### Aluminium alkoxide preparation-batch I

To 108 g of deionized water at 85°C was added 13.014 g AI(OC₄H₉)₃) while stirring. Subsequently, 7.8 ml of 1M HN0₃ was introduced, and the resulting solution (actually a colloidal dispersion) was aged for 12 hours at 85°C.

### Aluminum alkoxide preparation-batch II

The same procedure as above was-followed with the exception that the weight of Al(OC₄H₉)₃ was doubled.

### Silicon alkoxide preparation

To 104 g Si(OC₂H₅)₄ was added 90 g of absolute ethyl alcohol, followed by 9 g of deionized water and 1 drop of concentrated HN0₃.

Combining this hydrolyzed silicon alkoxide batch with batch I of the hydrolyzed aluminum alkoxide corresponded to a 90 Si0₂: 10 AI₂0₃ ratio on an oxide basis. The use of batch II of the hydrolyzed aluminum gave a 80 Si0₂:20 AI₂0₃ oxide ratio.

Generally, in most of the coating experiments better results were obtained with the addition of a wetting agent to the hydrolyzed alkoxide mixture to enhance the application of the coating on the simulated waste-glass spheroids (or other glass shapes). After considerable screening, Triton X-102, a Rohm and Haas product, was found to be most effective at a concentration of about 0.5 volume percent, although acceptable coatings were obtained with up to -2 v/o (% by volume).

A system, represented by Figure 1, was assembled which allowed either of the silicon-aluminum alkoxide mixtures to be atomized onto the waste-glass spheroids, followed by heating. This heating to cure the coating was performed as depicted in Figure 1, or alternatively, by preheating the spheroids to about 250°C before spray application of the coating. In this case a wetting agent (surfactant) was not required. Subsequent heating to 500°C removed all water of hydration and residual alkyls to yield an adherent, amorphous coating. Although the coating produced at 500°C was porous, the porosity was not joined and the coating served as a durable barrier against leaching. Heating to 800-850°C produced a totally dense, amorphous coating identical to that which would be obtained by melting at much higher temperatures using conventional processes.

The coating process was repeated a number of times to increase the thickness of the coating and to ensure against imperfections such as connected porosity or cracks. Even when the coating composition did not exactly match that of the spheroid, cracks or spalling of the coating due to differences in thermal expansion coefficients were not observed. Compositional analysis by EDAX across the spheroid-coating interface indicated some short-range "diffusion" of sodium in particular from the spheroid into the coating. Perhaps this is promoted by the reactivity, resembling chemical etching, of the alkoxides with respect to the glass spheroid (substrate).

### Example 2

The system illustrated in Figure 2 was built to enable the spheroids to be individually dispensed into the alkoxide coating fluid and, then, through a solution which caused curing of the coating into a stiff gel before the spheroids came into contact with one another. The two liquids were separated by an immiscible silicone-oil manufactured by Dow Corning Co. Using the silicon-aluminum batch II alkoxide mixture containing Triton surfactant prepared in Example 1 in the top of the column (Figure 2), and sodium hydroxide of about 0.5 M in the bottom segment, waste glass spheroids properly cleaned in trichloroethylene with ultrasonic agitation were successfully coated. The sodium hydroxide produced rapid and uniform curing of the coating. Other agents such as ammonium hydroxide, hydrochloric acid, and acetic acid required somewhat longer times for curing and, thus, a longer travel time in them was needed before the spheroids could be collected. Final heating to 500 or 800°C produced the quality vitreous coatings described in

### Example 1.

### Example 3

An alternative to using a "setting" agent in the bottom stage of the column in Figure 2, was to use a fluid which would cause curing of the coating by means of dehydration. Such a liquid was trichloroethylene or octanol or 2-ethyl-1 hexanol. The solubility of water in these fluids was sufficient, particularly when they were warmed to -75°C, to cause the coating to harden. Although the hardening did not occur as rapidly as with the sodium hydroxide setting agent, a high quality coating as described in Example 1 could nevertheless be obtained. In a continuous system, the water would be extracted by molecular sieve, for example, and circulated back to the column.

## Claims

1. A method of encapsulating glass or ceramic spheroids containing nuclear waste characterised by (A) dropping the spheroids individually into a coating apparatus; (B) coating the spheroids in the coating apparatus with a composition which comprises (1) from 30 to 85% by weight, calculated as Si0₂, of a partially hydrolyzed silicon compound having the general formula or where each R is independently selected from alkyl to e₁₀ and alkenyl to e₁ₒ, each R' is independently selected from R and aryl, each X is independently selected from chlorine and bromine, m is 0 to 3, n is 0 to 4, p is 0 to 1, and m+n+p equals 4; (2) up to about 30% by weight, calculated as A1₂0₃, of a partially hydrolyzed aluminium compound having the general formula or where each R is independently selected from alkyl to C₁₀ and alkenyl to C₁₀, each R' is independently selected from R and aryl, each X is independently selected from chlorine and bromine, q is 0 to 3, r is 0 to 3, s is 0 to 1, and q+r+s equals 3, and (3) from 30 to 50 percent by weight of an alcohol; (C) hardening the coatings on the spheroids whilst preventing the coated spheroids from touching one another; and (D) curing the coatings by heating the coated spheroids in air to a temperature of up to 850°C.

2. A method according to claim 1, characterised in that the spheroids are coated by spraying the composition onto them as they fall.

3. A method according to claim 2, characterized in that the coatings on the spheroids are hardened by heating them as they fall.

4. A method according to claim 1, characterized in that the spheroids are first heated to about 250°C and are coated by spraying the compositions onto them.

5. A method according to claim 1, characterized in that the spheroids are coated by dropping them into the composition.

6. A method according to claim 1, characterized in that the coatings on said spheroids are hardened by immersion in a setting agent.

7. A method according to claim 6, characterized in that the setting agent is an aqueous solution of MOH where M is selected from alkali metals, ammonium, and mixtures thereof.

8. A method according to claim 6 or 7, characterized in that the agent is heated to about 75°C.

9. A method according to claim 1, characterized in that the coatings on the spheroids are hardened by immersion in a dehydrating agent.

10. A method according to claim 9, characterized in that the dehydrating agent is trichloroethylene.

11. A method according to claim 9 or 10, characterized in that the dehydrating agent is heated to about 75°C.

12. A method according to claim 1, characterized in that the composition is hardened by coating the spheroids with a setting agent prior to coating thsm with the composition.

13. A method according to any of preceding claims, characterized in that the spheroids are from 1/2 to 25 mm in diameter.

14. A method according to any of the preceding claims, characterized in that steps (A), (B), (C) and (D) are repeated from 5 to 10 times.

15. A method according to claim 1, characterized in that the spheroids are coated and hardened by dropping them into a vessel containing the composition on top and a hardening fluid on the bottom, the composition and the hardening fluid being separated by an immiscible liquid.

16. A method according to claim 15, characterized in that the immiscible liquid is a silicon oil.

17. A method according to any of claims 1 to 16, characterized in that the coated spheroids are cured by heating to a temperature of from 400 to 500°C.

18. A method according to any of claims 1 to 17,' characterized in that prior to curing the coated spheroids are heated to a temperature of about 100°C.

## Revendications

1. Procédé pour encapsuler des sphéroïdes de verre ou de céramique contenant des déchets radioactifs, caractérisé en ce que (A), l'on fait tomber un par un les sphéroïdes dans un appareil de revêtement: (B) on revêt, dans cet appareil, les sphéroïdes avec une composition qui comprend (1) de 30 à 85% en poids, calculé en Si0₂ d'un composé du silicium partiellement hydrolysé répondant à la formule générale ou où chacun des R est choisi indépendamment entre les acoyls en C,, et les alcényls en Cₗₒ, chacun des R' est choisi indépendamment parmi les R et un aryl, chacun des X est choisi indépendamment entre le chlore et le brome, m est 0 à 3, n est 0 à 4, p est 0 à 1, et m+n+p est égal à 4, (2) jusqu'à 30% en poids, calculé en AI₂0₃, d'un composé de l'aluminium partiellement hydrolysé répondant à la formule générale ou, où chacun des R est choisi indépendamment parmi les alcoyls en e₁₀ et les alcényls en Cₗₒ, chaque R' est choisi indépendamment entre R et un aryl, chacun des X est choisi indépendamment entre le chlore et le brome, q est 0 à 3, r est 0 à 3 et s est 0 à 1, et q+r+s est égal à 3, et, (3) de 30 à 50% en poids d'un alcool; (C) l'on fair durcir les revêtements des sphéroïdes tout en évitant que les sphéroïdes revêtus se tournent les uns les autres; et (D) on polymèrise les revêtements en chauffant les sphéroïdes revêtus, dans l'air, à une température pouvant aller jusqu'à 850°C.

2. Procédé suivant la revendication 1, caractérisé en ce que les sphéroïdes sont revêtus, par pulvérisation sur eux, de la composition au moment de leur chute.

3. Procédé suivant la revendication 2, caractérisé en ce que le revêtement déposé sur les sphéroïdes est durci par chauffage pendant leur chute.

4. Procédé suivant la revendication 1, caractérisé en ce que les sphéroïdes sont d'abord chauffés à environ 250°C et sont revêtus en pulvérisant sur eux la composition.

5. Procédé suivant la revendication 1, caractérisé en ce que les sphéroïdes sont revêtus du fait qu'ils tombent dans la composition.

6. Procédé suivant la revendication 1, caractérisé en ce que les revêtements des sphéroïdes sont durcis par immersion dans un agent de fixation.

7. Procédé suivant la revendication 6, caractérisé en ce que l'agent de fixation est une solution aqueuse de MOH où M est choisi parmi les métaux alcalins, l'ammonium et leurs mélanges.

8. Procédé suivant les revendications 6 ou 7, caractérisé en ce que l'agent de fixation est chauffé à environ 75°C.

9. Procédé suivant la revendication 1, caractérisé en ce que les revêtements des sphéroïdes sont durcis par immersion dans un agent déshydratant.

10. Procédé suivant la revendication 9, caractérisé en ce que l'agent déshydratant est le trichloréthylène.

11. Procédé suivant la revendication 9 ou 10, caractérisé en ce que l'agent déshydratant est chauffé à environ 75°C.

12. Procédé suivant la revendication 1, caractérisé en ce que la composition est durcie en revêtant les sphéroïdes avec un agent de fixation avant de les revêtir avec la composition.

13. Procédé suivant l'une quelconque des revendications précédentes, caractérisé en ce que les sphéroïdes ont un diamètre de 0,5 à 25 mm.

14. Procédé suivant l'une des revendications précédentes, caractérisé en ce que les étapes (A), (B), (C), et (D) sont répétées jusqu'à 5 et dix fois.

15. Procédé suivant la revendication 1, caractérisé en ce que les sphéroïdes sont revêtues et durcies en tombant dans un récipient contenant la composition dans sa partie haute et un fluide durcissant dans sa partie inférieure, la composition et le fluide durcissant étant séparés par un liquide non-miscible.

16. Procédé suivant la revendication 15, caractérisé en ce que le liquide non-miscible est une huile de silicone.

17. Procédé suivant l'une quelconque des revendications 1 à 16, caractérisé en ce que les sphéroïdes revêtus sont polymérisés en les chauffant à une température entre 400 et 500°C.

18. Procédé suivant l'une quelconque des revendications 1 à 17, caractérisé en ce que les sphéroïdes revêtus sont chauffés, avant la polymérisation, à une température d'environ 100°C.

## Patentansprüche

1. Verfahren zur Umkapselung von aus Glas oder Keramik bestehenden Sphäroiden, die nuklearen Abfall enthalten, gekennzeichnet durch (A individuelles Fallenlassen der Sphäroide in ein Beschichtungsgerät; (B) Beschichten der Sphäroide in dem Beschichtungsgerät mit einer Zusammensetzung, die folgendes umfaßt: (1) 30 bis 85 Gew%, berechnet als Si0₂, eine teilweise hydrolisierten Siliziumverbindung mit der allgemeinen Formel oder wobei jedes R unabhängig ausgewählt ist aus Alkyl zu e₁₀ und Alkenyl zu Cᵢₒ, jedes R' unabhängig ausgewählt ist aus R und Aryl, jedes X unabhängig ausgewählt ist aus Chlor und Brom, m den Wert 0 bis 3 besitzt, n der Wert 0 bis 4 besitzt, p den Wert 0 bis 1 besitzt, und m+n+p gleich 4 ist; (2) bis zu etwa 30 Gew%, berechnet als AI_{z}0₃, einer teilweise hydrolisierten Aluminiumverbindung mit der allgemeinen Formel oder wobei jedes R unabhängig ausgewählt ist aus Alkyl bis e₁₀ und Alkenyl bis Cᵢₒ, jedes R' unabhängig ausgewählt ist aus R und Aryl, jedes X unabhängig ausgewählt ist aus Chlor und Brom, q den Wert 0 bis 3 besitzt, r den Wert 0 bis 3 besitzt, s den Wert 0 is 1 besitzt, und q+r+s gleich 3 ist, und (3) 30 bis 50 Gew% eines Akohols; (C) Erhärten der Beschichtungen auf den Sphäroiden, während die beschichteten Sphäroide daran gehindert werden, einander zu berühren; und (D) Aushärten der Beschichtungen durch Erhitzen der beschichteten Sphäroide in Luft bis auf eine Temperatur von 850°C.

2. Verfahren nach Anspruch 1, dadurch gekennzeichnet, daß die Sphäroide durch Aufsprühen der Zusammensetzung auf die Späroide während ihres Fallens beschichtet werden.

3. Verfahren nach Anspruch 2, dadurch gekennzeichnet, daß die Beschichtungen auf den Sphäroiden durch Erhitzen erhärtet werden, während diese Fallen.

4. Verfahren nach Anspruch 1, dadurch gekennzeichnet, daß die Sphäroide zuerst auf eine Temperatur von etwa 250°C erhitzt und dann durch Aufsprühen der Zusammensetzung auf die Sphäroide beschichtet werden.

5. Verfahren nach Anspruch 1, dadurch gekennzeichnet, daß die Sphäroide durch Fallenlassen in die Zusammensetzung beschichtet werden.

6. Verfahren nach Anspruch 1, dadurch gekennzeichnet, daß die Beschichtungen auf den Sphäroiden durch Eintauchen in ein Erhärtungsmittel erhärtet werden. ,

7. Verfahren nach Anspruch 6, dadurch gekennzeichnet, daß das Erhärtungsmittel eine wäßrige Lösung von MOH ist, wobei M ausgewählt ist aus Alkalimetallen, Ammonium und Mischungen davon.

8. Verfahren nach Anspruch 6 oder 7, dadurch gekennzeichnet, daß das Mittel auf etwa 75°C erhitzt wird.

9. Verfahren nach Anspruch 1, dadurch gekennzeichnet, daß die Beschichtungen auf den Sphäroiden durch Eintauchen in ein dehydrierendes Mittel erhärtet werden.

10. Verfahren nach Anspruch 9, dadurch gekennzeichnet, daß das dehydrierende Mittel Trichloroäthylen ist.

11. Verfahren nach Anspruch 9 oder 10, dadurch gekennzeichnet, daß das dehydrierende Mittel auf etwa 75°C erhitzt wird.

12. Verfahren nach Anspruch 1, dadurch gekennzeichnet, daß die Zusammensetzung erhärtet wird durch Beschichten der Sphäroide mit einem Erhärtungsmittel vor der Beschichtung der Sphäroide mit der Zusammensetzung.

13. Verfahren nach einem der vorhergehenden Ansprüche, dadurch gekennzeichnet, daß die Sphäroiden einen Durchmesser von 1/2 bis 25 mm aufweisen.

14. Verfahren nach einem der vorhergehenden Ansprüche, dadurch gekennzeichnet, daß die Schritte (A), (B), (C) und (D) 5 bis 10 mal wiederholt werden.

15. Verfahren nach Anspruch 1, dadurch gekennzeichnet, daß die Sphäroide durch ihr Fallenlassen in ein Gefäß beschichtet und erhärtet werden, welches die Zusammensetzung auf der Oberseite und eine erhärtende Flüssigkeit am Boden enthält, wobei die Zusammensetzung und die erhärtende Flüssigkeit durch eine unmischbare Flüssigkeit voneinander getrennt sind.

16. Verfahren nach Anspruch 15, dadurch gekennzeichnet, daß die unmischbare Flüssigkeit ein Silikonöl ist.

17. Verfahren nach einem der Ansprüche 1 bis 16, dadurch gekennzeichnet, daß die beschichteten Sphäroide durch Erhitzen auf eine Temperatur von 400 bis 500°C ausgehärtet werden.

18. Verfahren nach einem der Ansprüche 1 bis 17, dadurch gekennzeichnet, daß vor dem Aushärten die beschichteten Sphäroide auf eine Temperatur von etwa 100°C erhitzt werden.
